

Jan. 17, 1939.

F. L. BUCHANAN ET AL

2,143,840

PAPER STOCK

Filed Feb. 5, 1936



Fig. 1



Fig. 2



Fig. 3

## Inventors

Fred L. Buchanan and  
Reynolds Guyer

Canwell & Lagaard  
Attorneys

## UNITED STATES PATENT OFFICE

2,143,840

## PAPER STOCK

Fred L. Buchanan and Reynolds Guyer, St. Paul, Minn., assignors to Waldorf Paper Products Company, St. Paul, Minn., a corporation of Minnesota

Application February 5, 1936, Serial No. 62,452

3 Claims. (Cl. 92—39)

Our invention relates to paper stock and particularly to a light caliper paper stock used for forming cartons.

An object of the invention resides in providing 5 a light caliper paper stock which is opaque to the light rays tending to promote rancidity in butter and other fatty substances.

Another object of the invention resides in providing a paper stock which in addition to being 10 opaque to certain light rays has all of the other requirements of paper stock for cartons for butter and other fatty substances.

A still further object of the invention resides in providing a paper stock having the above noted 15 characteristics which will be no thicker than ordinary paper stock used for cartons for such purpose.

An object of the invention resides in providing 20 a paper stock having a body portion colored to render the same opaque to the light rays tending to promote rancidity in butter and other fatty substances and of a thickness less than that of the facing thereof.

A still further object of the invention resides 25 in providing a paper stock of the character desired in which bleeding through of the coloring of the body portion or discoloration thereby is prevented or obscured.

Another object of the invention resides in providing 30 a paper stock of the character desired having a liner of a thickness less than that producing opacity to light rays reflected from the coloring of the body portion and passing through the liner and in coloring the liner with a light 35 coloring adapted to obscure such light rays, and preferably a color complementing the color of the commodity contained within the carton.

An object of the invention resides in the 40 method of forming the paper stock.

Other objects of the invention reside in the 45 details of construction hereinafter illustrated and/or described and in the manner of performing and the order of performing the various steps of the method.

In the drawing:

Fig. 1 is a diagrammatic longitudinal elevational view of a cylinder type of paper making machine.

Fig. 2 is a plan view of a portion of a sheet 50 of paper stock constructed in accordance with our invention and with portions of the same cut away to illustrate the parts of the paper stock.

Fig. 3 is a cross sectional view of the paper 55 shown in Fig. 2 and drawn to an enlarged scale.

This application is a continuation in part of

our application for patent, Serial No. 749,389, filed Oct. 22, 1934 for Paper board.

In practice it has been found that light rays having certain wave lengths and particularly the shorter wave lengths have the effect of 5 promoting rancidity in butter and other similar fatty substances. Heretofore, wrappers constructed of metal foil, paper and other materials opaque to such light rays have been used in addition to the regular carton in which the substances are placed for the filtering out of such light rays. This involves additional expense and adds to the inconvenience of the packer as well 10 as the user. It has been applicants' problem to overcome this added expense and inconvenience 15 by providing a paper carton stock which would have in addition to the usual characteristics of such paper stock the added characteristic of filtering out the undesirable light rays. This applicants had to accomplish without appreciably 20 increasing the cost of the stock or without increasing the thickness thereof. Applicants solved the problem by the use of webs of suitable thickness and by the coloring of certain of the webs and by the arrangement thereof, as will 25 hereinafter be more fully described in detail.

For the purpose of illustrating the method of 30 constructing the invention, a portion of an ordinary cylinder type paper making machine has been shown in Fig. 1. This machine comprises a plurality of vats 11, 12, 13, 14, 15, 16 and 17 which have cylinders 21, 22, 23, 24, 25, 26 and 27 placed within the same. These cylinders are constructed of wire screen of a suitable mesh which depends upon the kind of fiber used in the stock 35 fed to the machine. Within these vats are disposed molds 28 which fit about the cylinders and lead the stock to the same. A number of suction pumps not shown, remove the water from within the cylinders, causing a small hydrostatic 40 head within the various vats which draws the paper stock to the outer surfaces of the cylinders.

Overlying each of the cylinders 21 to 27 are a number of couch rolls 29 which occupy the positions relative to said cylinders shown in the 45 drawing. A felt 30 passes between the rolls 29 and the various cylinders and picks off the webs of fibers deposited upon the surfaces of the screen cylinders through the hydrostatic action previously described. The various webs formed 50 on the cylinders 21, 22, 23, 24, 25, 26 and 27 are brought together upon the felt 30 and form the composite sheet which is indicated at 32. This sheet adheres to and is carried along with the felt 30, being disposed upon the underside of 55

the lower reach 31 of felt 30. The felt 30 is carried back over the last couch roll 29, the upper reach 41 thereof being supported on an upper roll 33. This brings the sheet 32 upon the upper surface of the reach 41 of said felt. A series of tensioning rolls 34, 35, 36 and 37 serve to maintain the proper tension in the felt 30.

Operating in conjunction with the felt 30 is another felt 38 which has a run 39 which overlies the return run 41 of the felt 30. This felt is supported on rolls 42, 43, 44 and 45 and is maintained in proper tension by means of rolls 46, 47 and 48.

The sheet 32 throughout the runs 39 and 41 of felts 38 and 30 passes between said felts and is run through a series of primary press rolls 51 and 52 which squeeze out a certain percentage of the water. From these rolls the sheet passes through a series of secondary press rolls, the first pair being indicated by the numerals 53 and 54. The felt 38 leaves the sheet 22 when the same passes the last roll 51 and is carried back through the tightener rolls 46, 47 and 48. This leaves the roll 53 to directly engage the upper surface of the sheet and to give a finish to the same. The sheet 32 after leaving rolls 53 and 54 is successively carried through a second pair of press rolls 55 and 56, a third pair of press rolls 57 and 58 and through a fourth pair of press rolls 61 and 62.

Operating in conjunction with the press rolls 55 and 56 is a felt 63 which is carried on rolls 64 and roll 56 and which comes into line contact with sheet 22 when in engagement with the roll 55. Tension rolls 65, 66 and 67 are employed for tensioning this felt. In a similar manner another felt 68 corresponding to felt 63 passes over roll 58 and comes into line contact with the sheet 22 when it engages roll 57. Felt 68 passes over rolls 71, 72, 73 and 74 and is tightened by means of tension rolls 75, 76 and 77. Passing between rolls 61 and 62 is another felt 78 similar to the felt 68. This felt is supported on rolls 81, 82 and 83 and is tensioned by means of rolls 84, 85 and 86. In the passage of the sheet through the secondary press rolls, one of the rolls of each pair directly engages the sheet so as to give a finish to the same. It will be noted that the sheet 22 passes through the rolls 57 and 58 in reverse order so that the sheet is finished on both sides thereof. It will further be noted that the first, second and fourth pairs of press rolls finish the sheet on the lowermost surface of the same when the sheet leaves the vats 11 to 17, thereby giving a finer finish to this portion of the sheet.

The sheet 22 on leaving the press rolls passes through one or more driers 87. These driers consist of heated rolls 88 which are arranged in staggered relation and over which the sheet alternately passes. As many of these driers are utilized as are necessary to properly dry the paper so that when the paper leaves the machine the same is ready to be cut in sheets or rolled in rolls as required.

Our improved paper stock as shown in Figs. 2 and 3 comprises a body portion 87, a facing 88 and a liner 89. These various parts will now be described in detail.

The body portion 87 consists of a suitable stock which is dyed black through any of a number of suitable dyes now available for the purpose. This stock may be made from ordinary waste paper or any other suitable fiber and need not be of the highest grade. The dye is preferably a black

or any other color, or of suitable light absorbing characteristics to exclude or absorb light rays ranging from 7500 Angstrom units through 2400 Angstrom units. A sulphur black aniline dye containing sodium sulphite may be used for the purpose. The thickness of the body 87 varies, depending upon the ultimate thickness of the stock. In a stock of approximately sixteen points thickness, the body 87 would have a thickness of two and one-fourth points.

The facing 88 is preferably white or some other suitable color which is considerably thicker than the body 87. This facing is preferably constructed in two parts designated by the reference numerals 91 and 92. The part 91 is formed entirely of bleached sulphite pulp. The part 92 consists of approximately seventy-five percent ground wood and twenty-five percent sulphite pulp. Where the board is to be approximately sixteen points, the portions 92 and 91 would be about four and one-half points each, making the total thickness of the facing 88 about nine points.

The liner 89 is constructed of a material similar to the facing 88. However, a fiber of as high a quality as that used for the facing need not be employed since the liner is not constructed to receive printing ink. A pulp consisting of fifty percent ground wood and fifty percent sulphite pulp will answer the purpose. In order to maintain the stock the desired thickness it becomes necessary to reduce the thickness of the liner 89 as compared with the thickness of the facing 88. Where the entire thickness of the board is approximately sixteen points, the thickness of the liner would have to be four and three-fourths points. Where a pulp such as specified is used, the coloring from the body 87 would bleed through or the said liner would be sufficiently transparent to show the coloring in the body portion 87 through the same. In order to eliminate this disadvantage a light coloring is used in the liner which obscures or renders invisible any bleeding of or showing of the coloring in the body portion 87. Where the body portion 87 is colored black, a light blue coloring may be used in the liner 89 which produces the desired effect.

The method of forming our improved paper stock on the machine shown in Fig. 1 is as follows:

The stock used for the liner 89 is placed in the two vats 16 and 17 and two webs 101 and 102 are formed therefrom by the cylinders 26 and 27 and deposited upon the felt 30. These two webs form in conjunction the liner 89. In the vat 15 is placed the stock forming the body portion 87. A single web 103 is formed from this stock which constitutes the body portion 87. The portion 92 of facing 88 is formed by the two cylinders 23 and 24 and the stock for the same is deposited in the vats 13 and 14. These two cylinders form webs 105 and 106. The portion 91 of the facing 88 is formed by the cylinders 21 and 22 and consists of two webs 107 and 108. The stock for these two webs is placed in the vats 11 and 12. As the process continues, the various webs are added one to the other and collected on and carried by the lower run 31 of felt 30. The composite sheet of paper formed by the various webs specified passes between the two felts 30 and 38 and through the various primary press rolls, the secondary press rolls and the driers of the paper making machine. When the stock leaves the papermaking machine the same will have been formed with the body portion 87 opaque to the undesirable light rays with the

facing 88 opaque to the coloring of the body 87 and the exposed surface thereof suitably finished to receive printing ink and with the liner 89 colored to obscure the coloring of the body 87. After 5 the sheet has been so formed, the same is run through a paraffin machine by means of which a coating 109 is placed upon the inner surface of the liner 89. If desired, the outer surface of the facing 88 may also be provided with a similar 10 coating of paraffin 110. Where both surfaces of the sheet are paraffined the printing on the sheet is first performed and the paraffining done afterwards. In the formation of the paper the various fibers of the various webs are interlocked and 15 the resulting sheet is a composite structure of substantially homogeneous character.

Paper stock used for cartons for fatty substances such as butter, lard, oleomargarine and the like, usually run from fourteen to eighteen 20 points in thickness. Where the stock is to be sixteen points, as referred to, the web 101 would be approximately two and one-half points, and the remaining webs approximately two and one-fourth points. It can readily be comprehended, 25 however, that the paper could be made on a machine having less cylinders than that described since thicker webs can be readily formed than those specified. Also the relative thicknesses of the webs can be varied so long as the ultimate 30 structure has the desired characteristics. An important feature of the invention resides in constructing the facing with a suitable surface for printing and at the same time render the same opaque to light rays reflected from the body portion. This requires a considerable thickness. In 35 order to hold down the ultimate thickness of the paper board, the body portion is made relatively thin and is rendered opaque to the undesirable light rays and at the same time the liner also has to be made so thin that the coloring of the body portion would show through. This is overcome by coloring the liner.

Our invention is used in the same manner as other paper stock from which containers of the 45 type referred to are constructed. The stock may be first printed and thereafter paraffined and the sheets cut into the desired blanks which may be scored and cut to form containers of any suitable type, size and construction. The particular construction of the paper stock constituting our invention does not affect the flexibility of the stock 50 nor any of the other characteristics which can be procured by the selection of materials suitable for the purpose.

Our invention is highly advantageous in that 55 our improved paper stock may be used in the customary manner to construct containers for the desired products without involving any particular precaution or change in the method of manufacturing and using such containers. With our invention the chemical action which causes

fatty substances to become rancid is greatly retarded so that such substances maintain their desired condition for a greater length of time than when kept in ordinary containers. Our improved paper stock can be produced at substantially the 5 same cost as any other paper stock so that the same can readily be substituted for other types of paper stock now in use for the purpose. Our paper stock can be formed of the same thickness as paper stock now used for the intended purpose 10 and is provided with a facing having a surface suitable for printing the same as ordinary paper stock. By coloring the liner in the manner specified, the bleeding of the die in the body portion or the appearance of the coloring from the same 15 through the liner may be obscured or rendered imperceptible. By the use of a suitable coloring in the liner, a dual function is performed. Where the container is to be used for butter, a blue and preferably a light blue coloring may be used for 20 enhancing the appearance of the butter.

Changes in the specific form of our invention, as herein disclosed, may be made within the scope of what is claimed without departing from the 25 spirit of our invention.

Having described our invention, what we claim as new and desire to protect by Letters Patent is:

1. A paper stock comprising a facing of sufficient thickness and density and having suitable color characteristics to reflect light rays, a body 30 portion of less thickness than said facing, said body portion having a coloring therein serving to cause said body portion to absorb light rays, and a liner of less thickness than said facing capable of reflecting light rays, said liner having sufficient coloring therein to obscure bleeding through 35 of the coloring in said body portion.

2. A paper stock comprising a facing of a thickness of about nine points, and constructed of a material such as to cause said facing to reflect 40 light rays, a body portion of a thickness of about two and one-quarter points and constructed of a material treated in such a manner as to absorb the light rays tending to promote rancidity in fatty substances, and a liner constructed of a material similar to that of said facing and of a thickness of about five and one-quarter points 45 and a blue coloring in said liner.

3. A paper stock comprising a body including a web having a dark coloring therein for rendering 50 said web opaque to the light rays tending to promote rancidity in fatty substances, four facing webs on one side of the body web and jointly forming an opaque facing, two liner webs on the other side of the body web, and similar to the facing web, and forming a liner of less opacity 55 than said facing, and a light coloring in said liner webs obscuring the coloring of said body web.

FRED L. BUCHANAN. 60  
REYNOLDS GUYER.